

1

2,739,125

## HIGH METAL CONTENT COMPLEX SALTS OF SULFONIC ACIDS AND MINERAL OIL COMPOSITIONS THEREOF

Herbert Myers, Haddonfield, and Ferdinand P. Otto, Woodbury, N. J., assignors to Socony Mobil Oil Company, Inc., a corporation of New York

No Drawing. Application September 4, 1952,  
Serial No. 307,923

22 Claims. (Cl. 252—33)

This invention relates to improved lubricating oil compositions for use in internal combustion engines. More particularly, it relates to a new class of detergent additives for such lubricating oils and to a method for their preparation.

It is well known that lubricating oils tend to deteriorate under the conditions of use in present day diesel and automotive engines with attendant formation of sludge, lacquer and resinous materials which adhere to the engine parts, particularly the piston ring grooves and skirts, thereby lowering the operating efficiency of the engine. To counteract the formation of these deposits, certain chemical additives have been found which when added to lubricating oils have the ability to keep the deposit-forming materials suspended in the oil, so that the engine is kept clean and in efficient operating condition for extended periods of time. These addition agents are known in the art as detergents or dispersants. Metal organic compounds are particularly useful in this respect. These metal organic compounds are considered to be effective on the basis of their metal contents, coupled with their solubility in the oil. Generally, it has been found that the oil-soluble metal organic compounds having the greater percentages of metal provide the better detergents. On this basis, it has been sought to provide detergent compounds having the highest possible metal content. Metal sulfonates, such as metal petroleum sulfonates, obtained by the sulfonation of petroleum oils and synthetic sulfonates obtained by the sulfonation of wax aryl compounds, such as wax benzenes and wax naphthalenes are recognized in the art as being particularly effective detergents for mineral lubricating oils. The present invention is concerned with the provision of a new class of metal sulfonates, hereinafter called "complex" metal sulfonates, which have exceptionally high metal contents and which are highly superior oil detergents. The metal contents of these new complex metal detergent salts range from about 140 to about 180 per cent higher than that of the corresponding "normal" salts, i. e., salts having metal contents equivalent to the acid-hydrogen contents of the respective sulfonic acids from which they are derived.

It is the object of this invention to provide a new class of complex metal sulfonate salts having exceptionally high metal contents. It is a further object to provide oil compositions containing relatively small amounts of these salts, which compositions are of high detergent character. Other and further objects will become apparent from the following description of the invention.

Broadly, the complex metal salts of this invention are prepared by a method which comprises (1) intimately contacting an oil, or hydrocarbon, solution of a sulfonic acid, in the presence of water, with (a) at least about 1.6 equivalents of a metal hydroxide, (b) at least about 0.6 equivalent of a metal formate and (c) at least about 0.6 equivalent of a metal carboxylate, other than a metal formate, said equivalents being based on the equivalent of acid-hydrogen in the sulfonic acid solution, (2) substantially completely dehydrating the reaction mixture

2

formed in step 1 to produce the complex metal salt product and (3) filtering off insoluble material.

A satisfactory procedure for carrying out the invention is as follows: An aqueous slurry of the three metal-containing reagents is first prepared. This slurry is then intimately contacted with the sulfonic acid at a temperature of from about 25° C. up to about 100° C. A diluent oil is required in the case of the synthetic type sulfonic acids in order to facilitate the reaction and the handling and filtration of the complex salt product. The synthetic sulfonic acids are, therefore, first dissolved in oil to form a solution of, say, from about 20 to about 60 per cent of the acid in the oil, this solution being contacted with the reagent slurry. The petroleum sulfonic acids are, of course, already diluted with oil, generally being present therein in amounts of from about 20 to about 60 per cent, and these acids, or sour oils, ordinarily require no addition of diluent oil for the purpose of the reaction with the metal-containing reagents. The contacting of the sulfonic acid (solution) with the reagent slurry is accomplished by slow addition of the slurry to the heated acid with constant stirring of the mixture thus formed. When the addition is completed, the mixture is dehydrated by raising the temperature up to about 120° C. and maintaining this temperature until the dehydration is complete. The dehydrated product is then filtered to remove excess salt reagent. The product thus obtained is an oil solution which usually contains from about 20 to about 60-75 per cent, more or less, of the complex salt. It will be appreciated that in the case of the synthetic type sulfonic acids other hydrocarbon solvents may be used for the reaction besides mineral oil, such as a light naphtha, xylene, toluene or the like, however, use of a petroleum oil is preferred since it need not be removed after the reaction, the oil solution thus obtained being directly blendable with the lubricating oil desired to be fortified with the complex salt product.

Although the aforescribed procedure is the one generally used, the manner and time of bringing the sulfonic acid solution and the metal compound reagents together may be varied without affecting the reaction, or yield of complex salt product obtained. Thus, the sulfonic acid solution may be added to the reagent slurry or the sulfonic acid can be first reacted with the metal hydroxide and then reacted with an aqueous solution of the metal formate and metal carboxylate. Also, the normal metal sulfonate may be reacted with a slurry of all three reagents, the slurry containing the equivalent amounts of metal hydroxide, metal formate and metal carboxylate. This and other modifications of the procedure of the invention will be obvious to those skilled in the art. Several different procedures for carrying out the process of the invention are given in the illustrative examples hereinafter presented. In all cases, however, it is essential in our method that a good dispersion of the reactants be obtained, that water be present and the dehydration be carried essentially to completion. It is also necessary that certain specified amounts of the metal hydroxide, metal formate and metal carboxylate reagents be present in the reaction with the sulfonic acid in order to provide the complex salts of the invention. The metal formate and the metal carboxylate may be supplied in the form of a mixture of metal hydroxide with formic and carboxylic acids. For example, when the three reagents are supplied in the form of metal salts, at least about 1.6 equivalents of metal hydroxide, at least about 0.6 equivalent of metal formate and at least about 0.6 equivalent of metal carboxylate are required per equivalent of acid-hydrogen in the sulfonic acid solution utilized. Where the formic acid and carboxylic acid are supplied, as such, to the reaction, however, the amount of metal hydroxide used is increased

to 2.8 equivalents in order to provide the necessary equivalents of metal in the reaction.

The necessity of the presence of water is illustrated by the fact that when dry calcium formate and calcium acetate are added to an oil solution of a normal calcium sulfonate and heated, subsequent analysis of the filtered oil shows no increase in the calcium content thereof. In general, it may be said that an amount of water equal to at least about 25 per cent, by weight, of total metal salt reagent utilized in the reaction is satisfactory. However, a larger amount of water may be used, the amount in each case being limited only by practical considerations, e. g., the type of sulfonic acid, the solubility of the metal salts, the feasibility of handling and length of time to dehydrate the product, etc.

The necessity of dehydrating the reaction mixture is illustrated by the fact that if the reaction mixture is not substantially completely dehydrated, but only refluxed for a few hours, the oil phase, when separated from the aqueous phase, shows a metal content equal only to the normal metal sulfonate. The dehydration step has been conducted under various conditions and it has been found that there is no definite limitation on the method of dehydrating, except for practical considerations. Generally, the dehydration is accomplished by heating at moderately elevated temperatures, i. e., from about 20° C. to about 120° C. for several hours. Although higher temperatures may be used, they are unnecessary. In those instances where the dehydration temperature reached 150° C., the metal content of the products obtained was only slightly higher (0.1 per cent) than where the temperature remained below about 100° C. The dehydration may be facilitated by blowing a gas, such as air or nitrogen, through the heated reaction mixture. It is generally preferred to filter the product at temperatures in the neighborhood of 100° C. since this temperature is high enough to keep the product quite fluid.

Due to the intricate nature of the complex metal salts thus produced, no chemical formula can be ascribed to them at this time. Neither is the manner of their formation precisely known. However, without intending to limit our invention by theoretical considerations, it is believed that our complex salts are formed via a two-step process in which the normal metal sulfonate is first formed by reaction with the metal hydroxide, the normal salt then being reacted further with the metal hydroxide-metal formate-metal carboxylate reagent during dehydration to yield the final product. The formation of the complex salt during dehydration is postulated on the basis of certain experimental observations. Thus, although an oil solution of complex metal sulfonate is obtained by interaction of a sulfonic acid with an aqueous solution of metal formate and metal acetate by substantially completely dehydrating the reaction mixture (i. e., removal of at least about 90 per cent of the water), if the oil phase is separated before such dehydration, the metal content corresponds only to that of a normal metal sulfonate. Also, indications of the formation of complexes between the metal compound reagents during dehydration are had from X-ray diffraction examination of the solid material obtained on evaporating an aqueous solution of (a) calcium formate and calcium acetate and (b) calcium hydroxide, calcium formate and calcium acetate. These analyses show no patterns that can be attributed to either calcium formate or calcium acetate, thus inferring the formation of different compounds. Also, X-ray analysis of excess solid material isolated from a normal calcium sulfonate-calcium formate-calcium acetate reaction mixture was found to be identical to the aforementioned solid derived from a water solution of the metal formate and metal acetate. Furthermore, it has been found that more metal can be incorporated into the sulfonate complex by using a mixture of metal acetate and metal formate than by using an equivalent amount of either salt alone. This is believed to be due to the formation of an acetate-

formate complex. Finally, since the presence of an appreciable amount of water is necessary in order to form our complex salts, ionization is apparently an essential factor in their formation.

We are aware that certain complex metal sulfonate salts, somewhat similar in nature to the complex metal sulfonate salts herein contemplated, have been shown heretofore in the grease art. Thus, several patents, viz. Zimmer et al., No. 2,444,790, and O'Halloran, Nos. 2,553,422 and 2,562,814, disclose complex sulfonate salts as gelling agents. These salts are formed by reaction of normal sulfonate salts with a low molecular weight acid salt, such as metal acetate. Our complex salts are distinguished from the complex salts of these patents by virtue of the fact that these latter salts are oil-insoluble and provide grease-like structures in the oil, whereas our complex salts are oil-soluble. Only one carboxylate reagent salt is utilized in the preparation of the prior art salts whereas our complex salts are prepared from a combination of a formate salt with another carboxylate salt. Our complex salts have much greater metal contents and are apparently of an entirely different configuration from those of the prior art. Accordingly, our complex salts are claimed herein as new compositions of matter.

The metal constituent of the metal hydroxide, metal formate and metal carboxylate (other than metal formate) reactants used in the preparation of our complex salts may be different metals, so that mixed metal complex salts, i. e., salts having more than a single metal constituent, may be successfully prepared and are contemplated herein. We have, in fact, prepared and tested complex salts containing two and three metal constituents and have found them to be highly effective detergents as shown in the examples presented hereinafter. Up to the present time, our work has extended only to the metal salts of those metals falling within group I and group II of the periodic table. However, it seems probable that reagent salts of other metals will also be found to be suitable for the invention. We have found that complex metal salts of the metals of group II of the periodic system, particularly the calcium, barium and magnesium salts and the mixed salts of these metals, provide outstanding detergents for lubricating oils.

The carboxylic acids, or salts thereof, suitable for the preparation of our complex metal salts are the aliphatic carboxylic acids other than formic acid having up to about 20 carbon atoms in the aliphatic portion thereof. The acid may be either saturated or unsaturated. It may also contain certain substituent groups, such as phenyl, hydroxy, halogen, amino or mercapto groups. As non-limiting examples, there may be mentioned acetic acid, chloroacetic acid, phenyl acetic acid, hydroxy acetic acid, glycine, thioglycolic acid, acrylic acid, propionic acid, butyric acid, butenic acid, valeric acid, heptylic acid, caproic acid, lauric acid, myristic acid, palmitic acid, oleic acid, stearic acid and the like. The lower molecular weight acids, such as acetic acid, are preferred however, since they provide complex salts having the higher proportions of metal per mol of complex salt.

As aforesaid, the sulfonic acids suitable for use in this invention include oil soluble petroleum sulfonic acids and synthetic alkaryl sulfonic acids, particularly those having higher molecular weights, i. e., from about 300 to about 800. These sulfonic acids may be produced by sulfonation of petroleum stocks or synthetic alkyl aromatic compounds, such as alkyl-substituted benzenes or naphthalenes wherein the alkyl groups attached to the aromatic ring contain at least about 8 carbon atoms, the wax-substituted benzenes and naphthalenes being particularly preferred. The petroleum sulfonic acids, also known as "sour oils," are those obtained in the treatment of petroleum oils, particularly refined, or semi-refined oils, with concentrated or fuming sulfuric acid, and which remain in the oil after settling out of sludge. These

sulfonic acids may be represented by the general formula



where R is one or more alkyl, alkaryl or aralkyl groups and the aromatic nucleus is a single or condensed ring or partially hydrogenated ring. Typical of such petroleum sulfonic acids are those utilized in Examples 2-6 below, viz., Sour Oil Treat 162, prepared from a furfural-refined Mid-Continent type heavy distillate stock (Stock A) and Sour Oil Treats 183, 189 and 193, prepared from a furfural-refined East Texas stock (Stock B). The properties of these two typical oil stocks are given in Table I and the properties of the several sour oils prepared therefrom are given in Table II. The manner of preparation of the sour oils is illustrated by Example 1 showing the preparation of Sour Oil Treat 183.

TABLE I

| Properties                            | Stock A | Stock B |
|---------------------------------------|---------|---------|
| Kin. Vis. @ 100° F.                   | 82.33   | 134.4   |
| Kin. Vis. @ 212° F.                   | 9.30    | 12.22   |
| Viscosity Index                       | 97      | 85      |
| Percent Sulfur                        | 0.23    | 0.23    |
| Spec. Gravity                         | 0.8833  | 0.8922  |
| A. P. I. Gravity                      | 28.7    | 27.1    |
| Pour, ° F.                            | 20      | 20      |
| Flash, ° F.                           | 435     | 480     |
| Fire, ° F.                            | 495     | 530     |
| Color, Lovibond                       | 38      | 42      |
| Color, ASTM                           | 5       | 7       |
| Viscosity Gravity Constant at 210° F. | 0.814   | 0.822   |

TABLE II

|                     | Sour Oil Treat No. |       |      |      |
|---------------------|--------------------|-------|------|------|
|                     | 162                | 183   | 189  | 193  |
| Total N. N.         | 24.1               | 33.0  | 32.1 | 29.9 |
| True N. N.          | 19.6               | 28.1  | 26.3 | 22.9 |
| Kin. Vis. @ 210° F. | 29.48              | 28.91 | 26.5 |      |
| Benzene Insolubles  | 0.07               | 1.9   | 1.8  |      |

## EXAMPLE 1

## Preparation of Sour Oil Treat 183

Thirty per cent by weight of 103 to 104% sulfuric acid was added over a period of  $\frac{1}{2}$  hour to an air-agitated charge oil (East Texas heavy waxy neutral), the reaction mixture being maintained at 90° to 135° F. Quench water (6 per cent by weight of charge oil) was then added over a  $\frac{1}{2}$ -hour period at a temperature of 115° to 150° F., followed by a 20-hour settling period at 160° F. The sludge and spent acid were withdrawn, and the product blown with air for 2 hours at 160° F. to remove the occluded sulfur dioxide. A final settling period of 21 hours at 160° F. was carried out to insure as complete a removal as possible of spent acid and sludge. The final product had a total N. N. of 33.0 and a true N. N. of 28.1 and was obtained in a yield of about 97 per cent by weight of the oil charged. The total N. N. designates the combined acidity of the sulfonic acid and residual sulfuric acid in the sour oil, while the true N. N. designates the acidity due to the sulfonic acid alone.

## Preparation of calcium-formate-acetate-sulfonate complex

In the following examples, procedures for the preparation of complex calcium sulfonate salts of the character contemplated by this invention are given in order to illustrate various aspects and modifications of the invention. The amounts of reagents, i. e., calcium hydroxide, calcium formate and calcium acetate utilized in Examples 2-6 are based on the "total" acidity of the sour oil, which, as aforesaid, includes minor amounts of free sulfuric acid present therein. Calculations on the amount

of calcium incorporated into the final product were based on the "true" acidity, a measure of the organic sulfonic acids present in the sour oil and are expressed in terms of the percentage excess calcium over the theoretical value for the normal calcium sulfonate.

## EXAMPLE 2

Four hundred grams of Sour Oil Treat 162 were placed in a 1-liter, four-necked, round-bottom flask equipped with a mechanical stirrer, thermometer, air inlet tube, reflux condenser and dropping funnel. The sour oil was heated with stirring and a moderate stream of air passing through it to approximately 75° C.

10 A reagent slurry, prepared by adding a solution of 4.7 grams (0.6 equivalent based on total acidity) of 98 per cent formic acid and 6.6 grams (0.6 equivalent) glacial acetic acid in a 50 ml. water to a slurry of 18.5 grams (2.8 equivalents) grease makers' lime (96 per cent calcium hydroxide) in 50 ml. water, was then added slowly 15 to the sour oil over a one-hour period from a dropping funnel while maintaining the reaction temperature at 70-75° C. The slurry was stirred from time to time to assure homogeneity. An additional 25 ml. of water was used to complete the transfer of reagents to the reaction mixture. When the addition of the reagent slurry to the sour oil was complete, the heat was increased and the water removed by means of a Dean-Stark take-off. The dehydration was completed in about 1½ hours with the temperature being regulated so as not to exceed about 20 25 30 35 40 120° C. The temperature was maintained for an additional hour after all the water was apparently removed in order to insure complete dryness. Sixteen grams (4 per cent by weight of sour oil) of "Hyflo" (a diatomaceous earth filter aid) were then added with stirring and the product filtered through an electrically heated Büchner funnel using filter paper precoated with "Hyflo," under a vacuum of approximately 150 mm. and a temperature of 80-100° C. The product filtered in about 45 minutes yielding 385 grams of a bright, brownish red oil.

## 45 Analysis of product:

Per cent calcium=1.78 (140 per cent in excess of normal salt).

Per cent sulfur=1.23

Kin. vis. @ 210° F.=23.35

45 The complex calcium petroleum sulfonates may also be prepared by adding the sour oil to the reagent slurry. This procedure is illustrated by Example 3.

## EXAMPLE 3

50 Four hundred grams of Sour Oil Treat 183 were added over a one-hour period to a mechanically agitated and air-blown slurry containing 125 ml. water, 25.4 grams (2.8 equivalents based on total acidity) of grease makers' lime, 713 grams (0.6 equivalent) 88 per cent formic acid and 8.5 grams (0.6 equivalent) glacial acetic acid. The temperature of the reaction mixture was maintained at 65°-75° C. during the addition. The dehydration was effected by gradually heating the reaction mixture to 115° C. while removing the water with a Dean-Stark take-off. To insure the complete removal of occluded water, the temperature was maintained at 115° C. for one hour. The filtration was carried out by stirring into the product 16 grams (4 percent by weight of sour oil charge) of "Hyflo" filter aid and filtering the mixture 55 60 65 through an electrically heated Büchner funnel using filter paper precoated with "Hyflo."

## Analysis of product:

Per cent calcium=2.39 (140 per cent in excess of normal salt).

70 The reactants can also be combined by first neutralizing the sour oil with calcium hydroxide and then adding an aqueous solution of calcium formate and calcium acetate. The latter salts may either be preformed or

obtained, *in situ*, by the reaction of calcium hydroxide and the appropriate acids. The first step can be accomplished by adding a slurry of calcium hydroxide to the sour oil as in Example 4, or, inversely adding the sour oil to the calcium hydroxide slurry as in Example 5.

#### EXAMPLE 4.

Four hundred grams of Sour Oil Treat 189 were placed in a 1-liter, four-necked, round bottom flask fitted with a mechanical stirrer, thermometer, air inlet tube, reflux condenser and addition funnel. The sour oil was heated, with stirring and with a moderate stream of air passing through it, to approximately 75° C. A slurry of 14.2 grams (1.6 equivalents based on total acidity) of grease makers' lime in 75 ml. water was then added over a one-hour period in small increments through the dropping funnel. This was followed by a 25 ml. water wash to complete the transfer of the slurry, and then by a dropwise addition of a solution containing 8.9 grams (0.6 equivalent) of calcium formate and 12.0 grams (0.6 equivalent) of calcium acetate monohydrate in 100 ml. water over a one-hour period at 70-75° C. The dehydration was effected by gradually heating the reaction mixture to 115° C. while removing the water with a Dean-Stark take-off. To insure the complete removal of occluded water, the temperature was maintained at 115° C. for one hour. The filtration was carried out by stirring into the product 16 grams (4 per cent by weight of the sour oil charge) of "Hyflo" filter aid and filtering this mixture through an electrically heated Büchner funnel using filter paper precoated with "Hyflo."

#### Analysis of product:

Per cent calcium=2.58 (160 per cent in excess of normal salt).

Per cent sulfur=1.59

Kin. vis. @ 210° F.=56.78

#### EXAMPLE 5

A slurry of 14.1 grams (1.6 equivalents based on total acidity) of grease makers' lime in 100 ml. water was charged into a 1-liter, four-necked, round-bottom flask equipped with a mechanical stirrer, thermometer, air inlet tube, dropping funnel and reflux condenser and heated with stirring and moderate air blowing to approximately 75° C. Four hundred grams of Sour Oil Treat 189 were added through the dropping funnel over a two-hour period with the reaction temperature being maintained at approximately 75° C. The resulting mixture was then heated at 80° C. for one-half hour after which a solution prepared by the reaction of 6.5 grams (0.6 equivalent) 98 per cent formic acid, 8.3 grams (0.6 equivalent) glacial acetic acid and 10.5 grams (1.2 equivalents) grease makers' lime in 100 ml. water was added dropwise over a one-hour period at about 75° C. The dehydration was effected by gradually heating the reaction mixture to 115° C. while removing the water with a Dean-Stark take-off. To insure the complete removal of occluded water, the temperature was maintained at 115° C. for one hour. The filtration was carried out by stirring into the product 16 grams (4 per cent by weight of sour oil charged) of "Hyflo" filter aid and filtering this mixture through an electrically heated Büchner funnel using filter paper precoated with "Hyflo."

#### Analysis of product:

Per cent calcium=2.47 (165 per cent in excess of normal salt).

Per cent sulfur=1.46

Kin. vis. @ 210° F.=52.57

It is not necessary to use a sulfonic acid as the starting material. Example 6 illustrates a procedure in which a normal calcium petroleum sulfonate was reacted with an aqueous slurry containing equivalent amounts of cal-

cium hydroxide, calcium formate and calcium acetate to yield a complex salt.

#### EXAMPLE 6

Four hundred grams of a normal calcium petroleum sulfonate prepared by the neutralization of Sour Oil Treat 193 and containing 0.86 per cent calcium was charged into a 1-liter, four-necked, round-bottom flask equipped with a mechanical stirrer, thermometer, air inlet tube, addition funnel and reflux condenser. The normal salt was heated to 75° C. with stirring and moderate air blowing. A slurry containing 5.4 grams (0.6 equivalent based on a theoretical total N. N.=32) grease makers' lime, 8.9 grams (0.6 equivalent) calcium formate and 12.1 grams (0.6 equivalent) calcium acetate monohydrate in 100 ml. water was then added over a one-hour period. The dehydration was effected by gradually heating the reaction mixture to 115° C. while removing the water with a Dean-Stark take-off. To insure the complete removal of occluded water, the temperature was maintained at 115° C. for one hour. The filtration was carried out by stirring into the product 16 grams (4 per cent by weight of sulfonate charged) of "Hyflo" filter aid and filtering this mixture through an electrically heated Büchner funnel using filter paper precoated with "Hyflo."

#### Analysis of product:

Per cent calcium=2.40 (180 per cent in excess of normal salt).

Per cent sulfur=1.42

Kin. vis. @ 210° F.=48.37

Potentiometric base No.=47

A typical synthetic alkyl-aryl sulfonic acid, viz., wax-benzene (2-12) sulfonic acid was prepared as shown in the following example.

#### EXAMPLE 7

##### Preparation of wax-benzene (2-12) sulfonic acid

A paraffin wax having an average of 24 carbon atoms per molecule and a melting point of 126° F. was chlorinated at a temperature of about 100° C. with chlorine gas until the weight of the wax had increased about 12 per cent. The chlorowax thus obtained was then blown with nitrogen to remove any occluded chlorine and hydrogen chloride.

A 1000-gram portion of the chlorowax was then mixed with 500 grams of benzene in a 3-necked flask equipped with a stirrer, reflux condenser and a thermometer. The mixture was heated to a temperature of 60° C. Aluminum chloride was then added slowly over a period of two hours. The addition of aluminum chloride was accompanied by a vigorous evolution of hydrogen chloride. The temperature was then raised to a temperature of 80° C. and held there for one hour. The excess benzene was then removed by inverting the reflux condenser and heating to a temperature of 116° C. Two hundred milliliters of benzene were thus recovered. The mixture was cooled to a temperature of 60° C. and then another 1000 grams of chlorowax were added slowly. After completing the addition of this chlorowax, the temperature was raised to 100° C. and held there for one hour. The product was allowed to stand overnight at a temperature of about 60° C., and then was separated from the sludge by decantation and filtered by suction through clay.

Seventeen hundred and thirty-eight grams of wax-benzene thus obtained were placed in a 3-necked flask equipped with a stirrer and a thermometer and heated to a temperature of 40° C. Eight hundred and sixty-nine grams of oleum (15 per cent SO<sub>3</sub>) were added slowly to the wax-benzene from a dropping funnel at a rate regulated to maintain the temperature below 50° C. The addition of oleum consumed about 3 hours. The mixture

was then stirred for an additional hour to ensure complete reaction. The mixture was then poured into 1000 milliliters of water and subsequently 1810 grams of mineral oil were added to the mixture. The mixture thus obtained was stirred thoroughly and then allowed to stand until the water separated into a layer. The water layer was then drained off. The product thus obtained was approximately a 50 per cent blend of wax-benzene sulfonic acid in mineral oil and had a neutralization number of 40.7.

It will be understood that a wax-benzene prepared according to the foregoing procedure in which a quantity of chlorowax containing 2 atomic proportions of chlorine and having a chlorine content of 12 per cent is reacted with 1 mol of benzene is designated "wax-benzene (2-12)." Similarly, "wax-benzene (3-10)" and "wax-benzene (1-10)" may also be prepared by the reaction of sufficient amounts of chlorinated wax, containing 10 per cent by weight of chlorine, to provide 3 atomic proportions and 1 atomic proportion of chlorine per mol of benzene, respectively, in the reaction and are useful in the invention. In general, the amount of chlorowax containing from about 10 to about 18 per cent by weight of chlorine used in the reaction is sufficient to supply between 1 and 4 atomic proportions of chlorine per mol of benzene used.

#### EXAMPLE 8

##### Preparation of complex formate-acetate calcium wax-benzene (2-12) sulfonate

Four hundred grams of wax-benzene (2-12) sulfonic acid, prepared in the manner of Example 7, and 150 grams of mineral oil (SUV of 100 sec. @ 100° F. acid-refined Mid-Continent) were charged into a 1-liter, four-necked, round-bottom flask equipped with a mechanical stirrer, air inlet tube, thermometer, reflux condenser and dropping funnel. The solution was heated with stirring and with a moderate stream of air passing through it to approximately 75° C. A slurry prepared by intermixing 35.1 grams (2.8 equivalents based on total acidity) grease makers' lime, 9.3 grams (0.6 equivalent) 98 per cent acetic acid and 11.8 grams (0.6 equivalent) glacial formic acid in 150 ml. water was added dropwise over a one-hour period. Dehydration was effected by gradually heating the reaction mixture to 115° C. for one hour. The filtration was carried out by stirring into the product 22 grams (4 per cent by weight of sour oil charged) of "Hyflo" filter aid and filtering the mixture through an electrically heated Büchner funnel using filter paper pre-coated with "Hyflo."

##### Analysis of product:

Per cent calcium=2.58 (120 per cent in excess of normal salt).

Per cent sulfur=1.80

Kin. vis. @ 210° F.=13.90

Potentiometric base No.=36

#### EXAMPLES 9-18

As stated hereinbefore, we have found that the use of about 1.6 equivalents of metal hydroxide, about 0.6 equivalent of metal formate and about 0.6 equivalent of the metal carboxylate, other than metal formate, provide the best results in the preparation of our complex metal salts, these amounts being based on the acid-hydrogen value of the crude sulfonic acid, i. e., the total N.N. It is to be understood, however, that these proportions may vary somewhat depending upon the residual sulfuric acid content of the particular sour oil or synthetic sulfonic acid used. This sulfuric acid content may vary in amount from about several per cent to 20-30 per cent of the total acid content in different sour oils and for the obtaining of optimum results the metal formate and carboxylate reagents can be varied proportionately i. e., they may be decreased with an increase in the sulfuric acid value and vice versa. Table III shows the results

obtained in a series of preparations of a calcium formate-acetate-sulfonate complex salt utilizing varying amounts of the reagent salts for reaction with Sour Oil Treat 183. It will be observed that variations from the preferred amounts of reagents for the most part caused a decrease in the calcium content of the final product and that where increases in the metal content of the complex salt were obtained such increases were not in proportion to the increase in calcium content of reagent used. The procedure used in all cases was that described in Example 2. Generally, the preferred proportions found for the calcium reagents are also applicable to the reagent salts of the other metals contemplated herein, however, we have found that some variation from these proportions in certain instances and in the case of certain metals provides products of higher metal content. Although in such instances, the use of the higher amounts of reagents usually cause difficulty in the filtration of the product, such variation in the amounts of reagents are deemed to be within the scope of our invention. Also, as aforesaid, some variation in the amount of metal salt reagent must be permitted depending upon the residual sulfuric acid content of the particular sulfonic acid utilized. The amounts of the reagent salts designated herein, therefore, actually represent about the least amounts which may be utilized for the successful preparation of the complex salt products having the high metal content contemplated herein, but are not the exact amounts to be used in any and all cases.

Various grades of lime, such as grease makers' lime, Bell-Mine chemical grade hydrated lime and chemically pure lime, may be used in preparing the complex calcium salts of this invention. However, grease makers' lime is preferred because of its high purity, small particle size and its property of being wet by oil.

##### Engine evaluation

To demonstrate the ability of the calcium-formate-acetate-sulfonate complex salts of the invention as oil detergents, a series of oil blends thereof were prepared and tested in the Lauson D-4A engine detergency test and in the CFR diesel D-21 detergency test. The base oil used in these tests contained 1.0 per cent of an antioxidant (Pinene-P<sub>2</sub>S<sub>5</sub> reaction product). The results are given in Tables IV and V. Example 4A in Table V was prepared from Sour Oil Treat 193 by the procedure illustrated in Example 4. This product gave the following analysis—

##### Analysis of product:

Per cent calcium=2.38 (165 per cent in excess of normal salt).

Kin. vis. @ 210° F.=49.5

Potentiometric base No.=34

##### Lauson D-4A detergency test

This test determines the effectiveness of the lubricating oil in preventing fouling as measured by the cleanliness of rings, lands, ring grooves and piston skirts. Cleanliness ratings are based on a scale of from 100 to 0, a 100 rating signifying a perfectly clean condition and a 0 rating representing the worst possible deposit condition. Bearing weight loss is also measured as supplemental data.

A single cylinder, 4-cycle, liquid cooled Lauson engine with splash lubrication and having copper-lead bearings is used. The operating conditions are as follows:

Oil temperature..... °F..... 225  
Jacket temperature..... °F..... 275

Speed..... R. P. M..... 1825

Brake load..... H. P..... 1.6

One-half throttle.

13-1 air-fuel ratio.

Oil added every 20 hours (one-gallon sample used).

The engine is inspected at the end of 20, 60 and 100 hours,

the duration of the test being 100 hours. The fuel used is a controlled "Mobilgas special" type blend gasoline (40 per cent thermal +30 per cent catalytically cracked +30 per cent straight run +2.5 cc. TEL/gal.).

#### Diesel (D-21) detergency test

This test determines the effectiveness of the lubricating oil in preventing piston deposits and top ring wear.

A single cylinder CFR, 4-cycle, super-charged, diesel engine is used. The operating conditions are as follows:

Oil temperature  $^{\circ}\text{F}$  175

Jacket temperature  $^{\circ}\text{F}$  212

Speed R. P. M. 1800

Brake load H. P. 7.5

Oil addition every 8 hours starting at 4 hours (1½ gal. sample used).

Heat input B. t. u./min. 1260

The duration of the test is 60 hours. The fuel used is a No. 2 fuel oil containing 1 per cent sulfur. The results are reported in terms of piston cleanliness ratings as in the D-4 test.

of the products. The per cent excess of metal incorporated in the complexes varied somewhat from metal to metal, but still ranged from about 100 per cent to 150 per cent.

The results obtained utilizing these complex salts in the CFR diesel D-21 detergency test are also given in Table VI.

#### EXAMPLES 25-31

A series of both bimetallic and trimetallic complex sulfonates were also prepared (Examples 25-31). The data concerning their preparation, their inspection and their ratings in the CFR diesel D-21 detergency test are given in Table VII.

#### EXAMPLES 32-42

As stated previously herein, it is possible to replace the metal acetate reactant with substituted acetate or other carboxylate type salts in the preparation of the complex salts of the invention. A number of such preparations are illustrated by Examples 31-39 in Table VIII. Mixtures of two such salts (or acids) may also be used.

TABLE III.—PREPARATION OF CALCIUM-FORMATE-ACETATE-SULFONATE COMPLEX SALT USING 400 GRAMS SOUR OIL TREAT 183 (TOTAL N. N.=33.0. TRUE N. N.=28.1)

| Example No. | Reagents (With 125 ml. Water) |             |           |             |                              |             | Analysis of Product |                   |                               |                     |         |
|-------------|-------------------------------|-------------|-----------|-------------|------------------------------|-------------|---------------------|-------------------|-------------------------------|---------------------|---------|
|             | Lime (Grease Makers)          |             | 98% HCOOH |             | Glacial CH <sub>3</sub> COOH |             | Percent Ca          | Percent Excess Ca | Potentiometric Total Base No. | Kinematic Viscosity |         |
|             | Wt., g.                       | Equivalents | Wt., g.   | Equivalents | Wt., g.                      | Equivalents |                     |                   |                               | 100° F.             | 210° F. |
| 9           | 25.4                          | 2.8         | 6.6       | 0.6         | 8.5                          | 0.6         | 2.39                | 141               | 47                            | 996                 | 58.18   |
| 10          | 24.0                          | 2.6         | 6.6       | 0.6         | 8.5                          | 0.6         | 2.25                | 127               | 34                            | 1,073               | 62.40   |
| 11          | 33.8                          | 3.75        | 6.6       | 0.6         | 8.5                          | 0.6         | 2.39                | 141               | 47                            | 886                 | 53.42   |
| 12          | 36.0                          | 3.9         | 6.6       | 0.6         | 8.5                          | 0.6         | 2.45                | 148               | 45                            | 860                 | 51.61   |
| 13          | 25.4                          | 2.8         | 8.0       | 0.7         | 10.2                         | 0.7         | 2.38                | 140               | -----                         | 1,083               | 62.67   |
| 14          | 27.7                          | 3.0         | 8.0       | 0.7         | 10.2                         | 0.7         | 2.50                | 152               | -----                         | 1,083               | 63.98   |
| 15          | 30.0                          | 3.2         | 8.0       | 0.7         | 10.2                         | 0.7         | 2.47                | 149               | -----                         | 1,070               | 63.94   |
| 16          | 23.1                          | 2.5         | 5.2       | 0.45        | 6.6                          | 0.45        | 2.14                | 115               | 36                            | 951.8               | 56.70   |
| 17          | 25.4                          | 2.8         | 3.3       | 0.3         | 12.7                         | 0.9         | 1.89                | 90                | 32                            | 637                 | 41.44   |
| 18          | 25.4                          | 2.8         | 9.9       | 0.9         | 4.2                          | 0.3         | 2.24                | 126               | 38                            | 654                 | 42.73   |

TABLE IV.—CFR DIESEL (D-21) TEST ON CALCIUM-FORMATE-ACETATE-SULFONATE COMPLEX

| Example No. | Description of Detergent |     |     |                                      |       |                      | CFR Diesel Test (1.0% S Fuel) Oil + 1.0% Antioxidant <sup>4</sup> |                                |                          |                   |                                |
|-------------|--------------------------|-----|-----|--------------------------------------|-------|----------------------|-------------------------------------------------------------------|--------------------------------|--------------------------|-------------------|--------------------------------|
|             | Sulfonic Acid            |     |     | Equivalents of Reagents <sup>1</sup> |       |                      | Percent Ca                                                        | Percent Excess Ca <sup>2</sup> | Percent Detergent in Oil | Percent Ca in Oil | Cleanliness Rating at 60 Hours |
|             |                          |     |     | Lime                                 | HCOOH | CH <sub>3</sub> COOH |                                                                   |                                |                          |                   |                                |
| 2           | Petroleum Treat 162      | 2.8 | 0.6 | 0.6                                  | 1.69  | 141                  | None                                                              | 3.5                            | 0.058                    | 62                | 85                             |
| 8           | Wax-Benzene (2-12)       | 2.8 | 0.6 | 0.6                                  | 2.58  | 120                  | 2.2                                                               | 0.058                          | 0.058                    | 85                | 85                             |

<sup>1</sup> Per equivalent of sulfonic acid, based on total N. N.

<sup>2</sup> Over that required for normal salt.

<sup>3</sup> S. A. E. 30 grade solvent-refined Mid-Continent oil.

<sup>4</sup> Pinene-P<sub>2</sub>S<sub>5</sub> product.

TABLE V.—LAUSON (D-4A) TEST ON CALCIUM-FORMATE-ACETATE-SULFONATE COMPLEX

| Example No. | Description of Detergent |     |     |                                      |                       |                                      | Lauson D-4A Test Oil <sup>3</sup> + 1.0% Antioxidant <sup>4</sup> |                                |                          |                   |                                 |
|-------------|--------------------------|-----|-----|--------------------------------------|-----------------------|--------------------------------------|-------------------------------------------------------------------|--------------------------------|--------------------------|-------------------|---------------------------------|
|             | Sulfonic Acid            |     |     | Equivalents of Reagents <sup>1</sup> |                       |                                      | Percent Ca                                                        | Percent Excess Ca <sup>2</sup> | Percent Detergent in Oil | Percent Ca in Oil | Cleanliness Rating at 100 Hours |
|             |                          |     |     | Lime                                 | Ca(HCOO) <sub>2</sub> | Ca(CH <sub>3</sub> COO) <sub>2</sub> |                                                                   |                                |                          |                   |                                 |
| 4-A         | Petroleum                | 2.8 | 0.6 | 0.6                                  | 2.38                  | 165                                  | None                                                              | 2.4                            | 0.058                    | 76                | 85                              |
| 4-A         | do                       | 2.8 | 0.6 | 0.6                                  | 2.38                  | 165                                  | 2.7                                                               | 0.088                          | 0.088                    | 85                | 85                              |

<sup>1</sup> Per equivalent of sulfonic acid, based on total N. N.

<sup>2</sup> Over that required for normal salt.

<sup>3</sup> S. A. E. 20 grade solvent-refined Pennsylvania oil (kin. vis. @ 100° F.=63, K. V. @ 210° F.=8.3).

<sup>4</sup> Pinene-P<sub>2</sub>S<sub>5</sub> product.

#### EXAMPLES 19-24

A number of metal complex salts of metals other than calcium which we have prepared are shown in Table VI. The table shows the mode of preparation and the analyses.

Examples 40-42, Table IX, illustrate this type of product. The results of CFR diesel engine D-21 detergency tests conducted on oil blends of the complex salt products thus obtained are included in the respective tables.

TABLE VI.—PREPARATION OF COMPLEX FORMATE ACETATE SULFONATES OTHER THAN CALCIUM AND THEIR ENGINE EVALUATION

| Example No.                                                                            | Description of Procedure |             |            |          |                                        |          |        |                       |          |        |                                                         |       |         |    |
|----------------------------------------------------------------------------------------|--------------------------|-------------|------------|----------|----------------------------------------|----------|--------|-----------------------|----------|--------|---------------------------------------------------------|-------|---------|----|
|                                                                                        | Sulfonic Acid            |             |            |          | Hydroxide                              |          |        |                       | Formate  |        |                                                         |       | Acetate |    |
|                                                                                        | Treat                    | Total N. N. | True N. N. | Wt. (g.) |                                        | Wt. (g.) | Equiv. |                       | Wt. (g.) | Equiv. |                                                         | (g.)  | Equiv.  |    |
| 19                                                                                     | 183                      | 33.0        | 28.1       | 400      | Mg(OH) <sub>2</sub>                    | 19.5     | 2.8    | HCOOH (88%)           | 7.3      | 0.6    | CH <sub>3</sub> COOH (glacial)                          | 8.4   | 0.6     |    |
| 20                                                                                     | Wax                      | 45.6        | 43.0       | 400      | Mg(OH) <sub>2</sub>                    | 26.4     | 2.8    | HCOOH (98%)           | 9.2      | 0.6    | CH <sub>3</sub> COOH (glacial)                          | 11.7  | 0.6     |    |
| 21                                                                                     | Ben-                     |             |            |          |                                        |          |        |                       |          |        |                                                         |       |         |    |
| 22                                                                                     | zene-                    |             |            |          |                                        |          |        |                       |          |        |                                                         |       |         |    |
| 23                                                                                     | (2-12).                  |             |            |          |                                        |          |        |                       |          |        |                                                         |       |         |    |
| 21                                                                                     | 183                      | 33.0        | 28.1       | 400      | Ba(OH) <sub>2</sub> ·8H <sub>2</sub> O | 106      | 2.8    | HCOOH (88%)           | 7.3      | 0.6    | CH <sub>3</sub> COOH (glacial)                          | 8.4   | 0.6     |    |
| 22                                                                                     | 193                      | 29.9        | 22.9       | 800      | Sr(OH) <sub>2</sub>                    | 43.0     | 1.6    | Sr(HCOO) <sub>2</sub> | 22.7     | 0.6    | Sr(CH <sub>3</sub> COO) <sub>2</sub> ·½H <sub>2</sub> O | 27.2  | 0.6     |    |
| 23                                                                                     | 189                      | 32.1        | 26.3       | 400      | ZnO                                    | 26.1     | 2.8    | HCOOH (98%)           | 6.4      | 0.6    | CH <sub>3</sub> COOH (glacial)                          | 8.2   | 0.6     |    |
| 24                                                                                     | 193                      | 29.9        | 22.9       | 800      | KOH                                    | 38.2     | 1.6    | HCOOK                 | 21.4     | 0.6    | CH <sub>3</sub> COOK                                    | 25.0  | 0.6     |    |
| Example No.                                                                            |                          |             |            |          |                                        |          |        |                       |          |        |                                                         |       |         |    |
| Description of Procedure                                                               |                          |             |            |          |                                        |          |        |                       |          |        |                                                         |       |         |    |
| Analysis                                                                               |                          |             |            |          |                                        |          |        |                       |          |        |                                                         |       |         |    |
| CFR Diesel Test (D-21) (1% S Fuel)<br>Oil <sup>2</sup> + 1.0% Antioxidant <sup>3</sup> |                          |             |            |          |                                        |          |        |                       |          |        |                                                         |       |         |    |
| Prepara-                                                                               |                          |             |            |          |                                        |          |        |                       |          |        |                                                         |       |         |    |
| Metal                                                                                  |                          |             |            |          |                                        |          |        |                       |          |        |                                                         |       |         |    |
| Percent                                                                                |                          |             |            |          |                                        |          |        |                       |          |        |                                                         |       |         |    |
| Percent Excess                                                                         |                          |             |            |          |                                        |          |        |                       |          |        |                                                         |       |         |    |
| Percent S                                                                              |                          |             |            |          |                                        |          |        |                       |          |        |                                                         |       |         |    |
| K. V. @ 210° F.                                                                        |                          |             |            |          |                                        |          |        |                       |          |        |                                                         |       |         |    |
| Potentiometric Total Base No.                                                          |                          |             |            |          |                                        |          |        |                       |          |        |                                                         |       |         |    |
| Percent Detergent in Oil                                                               |                          |             |            |          |                                        |          |        |                       |          |        |                                                         |       |         |    |
| Percent Metal <sup>1</sup> in Oil                                                      |                          |             |            |          |                                        |          |        |                       |          |        |                                                         |       |         |    |
| Cleanliness Rating at 60 Hours                                                         |                          |             |            |          |                                        |          |        |                       |          |        |                                                         |       |         |    |
| 19                                                                                     | 2                        | 1.55        | 155        |          | 1.84                                   | 63.19    |        | 23                    |          |        | None                                                    | 2.3   | 0.036   | 62 |
| 20                                                                                     | 4                        | 1.99        | 120        |          | 2.32                                   | 90.1     |        | 46                    |          |        | 2.32                                                    | 1.8   | 0.036   | 83 |
| 21                                                                                     | 2                        | 7.46        | 120        |          | 1.70                                   | 57.71    |        |                       |          |        | 2.7                                                     | 0.20  |         | 82 |
| 22                                                                                     | 4                        | 3.51        | 100        |          | 1.55                                   | 37.20    |        | 20                    |          |        | 3.6                                                     | 0.13  |         | 84 |
| 23                                                                                     | 2                        | 3.69        | 145        |          | 1.59                                   | 57.8     |        | 27                    |          |        | 2.6                                                     | 0.096 |         | 83 |
| 24                                                                                     | 4                        | 3.0         | 100        |          | 1.34                                   | 41.4     |        | 22                    |          |        | 3.9                                                     | 0.12  |         | 83 |

<sup>1</sup> Equivalent to 0.2% barium.<sup>2</sup> S. A. E. 30 grade solvent-refined Mid-Continent oil (kin. vis. @ 100° F. = 121, kin. vis. @ 210° F. = 12.2).<sup>3</sup> Pinene-P<sub>2</sub>S<sub>5</sub> reaction product.

TABLE VII.—PREPARATION OF BI AND TRI METALLIC COMPLEX ACETATE-FORMATE-SULFONATES AND THEIR ENGINE EVALUATION

| Example No.                                                                    | Description of Procedure |             |            |          |                           |          |        |                       |          |        |                                                         |          |         |    |
|--------------------------------------------------------------------------------|--------------------------|-------------|------------|----------|---------------------------|----------|--------|-----------------------|----------|--------|---------------------------------------------------------|----------|---------|----|
|                                                                                | Sulfonic Acid            |             |            |          | Hydroxide                 |          |        |                       | Formate  |        |                                                         |          | Acetate |    |
|                                                                                | Treat                    | Total N. N. | True N. N. | Wt. (g.) |                           | Wt. (g.) | Equiv. |                       | Wt. (g.) | Equiv. |                                                         | Wt. (g.) | Equiv.  |    |
| 25                                                                             | 193                      | 29.9        | 22.9       | 800      | Ca(OH) <sub>2</sub> (96%) | 26.3     | 1.6    | Mg(HCOO) <sub>2</sub> | 14.6     | 0.6    | Mg(CH <sub>3</sub> COO) <sub>2</sub> ·4H <sub>2</sub> O | 28.5     | 0.6     |    |
| 26                                                                             | 193                      | 29.9        | 22.9       | 800      | Mg(OH) <sub>2</sub>       | 19.8     | 1.6    | Ca(HCOO) <sub>2</sub> | 16.6     | 0.6    | Mg(CH <sub>3</sub> COO) <sub>2</sub> ·4H <sub>2</sub> O | 28.5     | 0.6     |    |
| 27                                                                             | 193                      | 29.9        | 22.9       | 800      | Mg(OH) <sub>2</sub>       | 19.8     | 1.6    | Ca(HCOO) <sub>2</sub> | 16.6     | 0.6    | Ca(CH <sub>3</sub> COO) <sub>2</sub> ·H <sub>2</sub> O  | 22.4     | 0.6     |    |
| 28                                                                             | 189                      | 32.1        | 26.3       | 400      | Ba(OH) <sub>2</sub>       | 31.8     | 1.6    | Ca(HCOO) <sub>2</sub> | 8.9      | 0.6    | Mg(CH <sub>3</sub> COO) <sub>2</sub> ·2H <sub>2</sub> O | 14.7     | 0.6     |    |
| 29                                                                             | 193                      | 29.9        | 22.9       | 800      | Ca(OH) <sub>2</sub> (96%) | 26.3     | 1.6    | Ba(HCOO) <sub>2</sub> | 28.9     | 0.6    | Mg(CH <sub>3</sub> COO) <sub>2</sub> ·4H <sub>2</sub> O | 27.6     | 0.6     |    |
| 30                                                                             | 193                      | 29.9        | 22.9       | 800      | Mg(OH) <sub>2</sub>       | 19.8     | 1.6    | Ca(HCOO) <sub>2</sub> | 16.6     | 0.6    | Ba(CH <sub>3</sub> COO) <sub>2</sub>                    | 25.4     | 0.6     |    |
| 31                                                                             | 25% diluted 193          | 22.5        | 17.2       | 800      | ZnO                       | 20.8     | 1.6    | Ca(HCOO) <sub>2</sub> | 12.4     | 0.6    | Ba(CH <sub>3</sub> COO) <sub>2</sub>                    | 24.5     | 0.6     |    |
| Example No.                                                                    |                          |             |            |          |                           |          |        |                       |          |        |                                                         |          |         |    |
| Description of Procedure                                                       |                          |             |            |          |                           |          |        |                       |          |        |                                                         |          |         |    |
| Analysis                                                                       |                          |             |            |          |                           |          |        |                       |          |        |                                                         |          |         |    |
| CFR Diesel (D-21) (1% S Fuel) Oil <sup>2</sup> + 1.0% Antioxidant <sup>3</sup> |                          |             |            |          |                           |          |        |                       |          |        |                                                         |          |         |    |
| Prepara-                                                                       |                          |             |            |          |                           |          |        |                       |          |        |                                                         |          |         |    |
| Metal                                                                          |                          |             |            |          |                           |          |        |                       |          |        |                                                         |          |         |    |
| Percent Metal                                                                  |                          |             |            |          |                           |          |        |                       |          |        |                                                         |          |         |    |
| Percent Excess Metal                                                           |                          |             |            |          |                           |          |        |                       |          |        |                                                         |          |         |    |
| Percent S                                                                      |                          |             |            |          |                           |          |        |                       |          |        |                                                         |          |         |    |
| K. V. @ 210° F.                                                                |                          |             |            |          |                           |          |        |                       |          |        |                                                         |          |         |    |
| Potentiometric Total Base No.                                                  |                          |             |            |          |                           |          |        |                       |          |        |                                                         |          |         |    |
| Percent Detergent in Oil                                                       |                          |             |            |          |                           |          |        |                       |          |        |                                                         |          |         |    |
| Percent Metal <sup>1</sup> in Oil                                              |                          |             |            |          |                           |          |        |                       |          |        |                                                         |          |         |    |
| Cleanliness Rating at 60 Hours                                                 |                          |             |            |          |                           |          |        |                       |          |        |                                                         |          |         |    |
| 26                                                                             | Example 4                | Ca=1.07     | 135        |          | 1.32                      | 46.6     |        | 33                    |          |        | None                                                    | 3.2      |         | 62 |
| 26                                                                             | do                       | Mg=0.46     | 155        |          | 1.38                      | 56.5     |        | 36                    |          |        | 2.9                                                     |          |         | 84 |
| 27                                                                             | do                       | Mg=0.61     | 155        |          | 1.46                      | 49.9     |        | 36                    |          |        | 2.9                                                     |          |         | 86 |
| 28                                                                             | do                       | Ba=4.08     | 120        |          | 1.54                      | 45.3     |        | 27                    |          |        | 3.0                                                     |          |         | 84 |
| 29                                                                             | do                       | Ba=1.15     | 130        |          | 1.38                      | 44.0     |        | 31                    |          |        | 3.2                                                     |          |         | 85 |
| 30                                                                             | do                       | Mg=0.25     | 165        |          | 1.55                      | 45.5     |        | 30                    |          |        | 3.8                                                     |          |         | 85 |
| 31                                                                             | do                       | Ba=1.57     | 190        |          | 1.22                      |          |        |                       |          |        | 3.4                                                     |          |         | 82 |

<sup>1</sup> Metal in oil equivalent to 0.2% barium.<sup>2</sup> S. A. E. 30 grade solvent-refined Mid-Continent oil (kin. vis. @ 100° F. = 121, kin. vis. @ 210° F. = 12.2).<sup>3</sup> Pinene-P<sub>2</sub>S<sub>5</sub> reaction product.

TABLE VII.—PREPARATION OF COMPLEX CALCIUM SULFONATES AND ENGINE EVALUATION

| Example No. | DESCRIPTION OF PROCEDURE |             |            |          |          |        |           |        |                     |          |        |                |
|-------------|--------------------------|-------------|------------|----------|----------|--------|-----------|--------|---------------------|----------|--------|----------------|
|             | Sulfonic Acid            |             |            |          | Lime     |        | 98% HCOOH |        | Name                | Wt. (g.) | Equiv. | Procedure used |
|             | Treat                    | Total N. N. | True N. N. | Wt. (g.) | Wt. (g.) | Equiv. | Wt. (g.)  | Equiv. |                     |          |        |                |
| 32          | 189                      | 32.1        | 26.3       | 400      | 24.7     | 2.8    | 6.5       | 0.6    | Chloroacetic Acid   | 13.0     | 0.6    | 32             |
| 33          | 189                      | 32.1        | 26.3       | 400      | 24.7     | 2.8    | 6.5       | 0.6    | Glycine             | 10.3     | 0.6    | 32             |
| 34          | 189                      | 32.1        | 26.3       | 400      | 24.7     | 2.8    | 6.5       | 0.6    | Glycolic Acid (70%) | 14.9     | 0.6    | 32             |
| 35          | 193                      | 29.9        | 22.9       | 400      | 23.0     | 2.8    | 5.9       | 0.6    | Thioglycolic Acid   | 11.8     | 0.6    | 32             |
| 36          | 182                      | 24.1        | 19.6       | 400      | 18.5     | 2.8    | 4.8       | 0.6    | Propionic Acid      | 7.6      | 0.6    | 32             |
| 37          | 193                      | 29.9        | 22.9       | 800      | 46.0     | 2.8    | 12.0      | 0.6    | Lactic Acid (85%)   | 13.5     | 0.6    | 32             |
| 38          | 25% Oil Diluted 193      | 22.5        | 17.2       | 800      | 33.1     | 2.8    | 9.0       | 0.6    | Crotonic Acid       | 16.5     | 0.6    | 32             |
| 39          | 162                      | 24.1        | 19.6       | 400      | 18.5     | 2.8    | 4.8       | 0.6    | Heptylic Acid       | 13.4     | 0.6    | 32             |

  

| Example No. | Analysis |                |        |                 |                               |                  |                          |                   | CFR Diesel Test (1.0% S Fuel)<br>Oil <sup>1</sup> +1.0% Antioxidant <sup>2</sup> |  |  |
|-------------|----------|----------------|--------|-----------------|-------------------------------|------------------|--------------------------|-------------------|----------------------------------------------------------------------------------|--|--|
|             | Calcium  |                | Sulfur | K. V. @ 210° F. | Potentiometric Total Base No. | Miscellaneous    | Percent Detergent in Oil | Percent Ca In Oil | Cleanliness Rating at 60 Hours                                                   |  |  |
|             | Percent  | Percent Excess |        |                 |                               |                  |                          |                   |                                                                                  |  |  |
| 32          | 2.89     | 158            | 1.67   | 48.0            |                               | Cl=1.05% N=0.48% | None                     | 0.058             | 62                                                                               |  |  |
| 33          | 2.35     | 156            | 1.68   | 70.78           |                               |                  | 2.4                      | 0.058             | 82                                                                               |  |  |
| 34          | 2.02     | 120            | 1.55   | 39.95           |                               |                  | 2.5                      | 0.058             | 84                                                                               |  |  |
| 35          | 1.52     | 85             | 2.05   | 38.97           | 18                            |                  | 3.8                      | 0.058             | 84                                                                               |  |  |
| 36          | 1.93     | 178            | 1.25   | 56.6            | 34                            |                  | 3.0                      | 0.058             | 85                                                                               |  |  |
| 37          | 2.14     | 150            | 1.49   | 128.4           | 34                            |                  | 2.7                      | 0.058             | 82                                                                               |  |  |
| 38          | 1.44     | 135            | 1.17   | 220.6           | 23                            |                  | 4.0                      | 0.058             | 85                                                                               |  |  |
| 39          | 1.98     | 186            | 1.27   | 200             | 35                            |                  | 3.0                      | 0.058             | 86                                                                               |  |  |

<sup>1</sup> S. A. E. 30 grade solvent refined Mid-Continent oil (kin. vis. @ 100° F. = 121; kin. vis. @ 210° F. = 12.2).<sup>2</sup> Pinene-P<sub>2</sub>S<sub>5</sub> reaction product.

TABLE IX.—PREPARATION OF COMPLEX CALCIUM-SULFONATES WITH THREE CONSTITUENTS AND THEIR ENGINE EVALUATION

| Example No. | Description Of Procedure |             |            |          |          |        |           |        |                         |          |        |                |
|-------------|--------------------------|-------------|------------|----------|----------|--------|-----------|--------|-------------------------|----------|--------|----------------|
|             | Sulfonic Acid            |             |            |          | Lime     |        | 98% HCOOH |        | Substituted Acetic Acid |          |        | Procedure Used |
|             | Treat                    | Total N. N. | True N. N. | Wt. (g.) | Wt. (g.) | Equiv. | Wt. (g.)  | Equiv. | Name                    | Wt. (g.) | Equiv. |                |
| 40          | 193                      | 29.9        | 22.9       | 800      | 46.0     | 2.8    | 12.0      | 0.6    | Lactic Acid (85%)       | 13.4     | 0.3    | 32             |
| 41          | 193                      | 29.9        | 22.9       | 800      | 46.0     | 2.8    | 12.0      | 0.6    | Chloroacetic Acid       | 12.0     | 0.3    | 32             |
| 42          | 25% Oil Diluted 193      | 22.5        | 17.2       | 500      | 21.6     | 2.8    | 5.6       | 0.6    | Glycine                 | 9.5      | 0.3    | 32             |
|             |                          |             |            |          |          |        |           |        | Heptylic Acid           | 16.5     | 0.3    |                |
|             |                          |             |            |          |          |        |           |        | Acetic Acid             | 4.8      | 0.4    |                |
|             |                          |             |            |          |          |        |           |        | Crotonic Acid           | 3.4      | 0.2    |                |

  

| Example No. | Analysis |                |        |                 |                               |               |                          |                   | CFR Diesel Test (1.0% S Fuel)<br>Oil <sup>1</sup> +1.0% Antioxidant <sup>2</sup> |  |  |
|-------------|----------|----------------|--------|-----------------|-------------------------------|---------------|--------------------------|-------------------|----------------------------------------------------------------------------------|--|--|
|             | Calcium  |                | Sulfur | K. V. @ 210° F. | Potentiometric Total Base No. | Miscellaneous | Percent Detergent In Oil | Percent Ca In Oil | Cleanliness Rating At 60 Hours                                                   |  |  |
|             | Percent  | Percent Excess |        |                 |                               |               |                          |                   |                                                                                  |  |  |
| 40          | 1.99     | 140            | 1.49   | 52.3            | 31                            | Cl=0.41       | None                     | 0.058             | 62                                                                               |  |  |
| 41          | 2.10     | 152            | 1.48   | 58.0            | 35                            |               | 2.9                      | 0.058             | 83                                                                               |  |  |
| 42          | 1.34     | 120            | 1.23   | 23.73           | 23                            |               | 2.8                      | 0.058             | 85                                                                               |  |  |
|             |          |                |        |                 |                               |               | 4.3                      | 0.058             | 82                                                                               |  |  |

<sup>1</sup> S. A. E. 30 grade solvent refined Mid-Continent oil (kin. vis. @ 100° F. = 121; kin. vis. @ 210° F. = 12.2).<sup>2</sup> Pinene-P<sub>2</sub>S<sub>5</sub> reaction product.

In the preparation of the product salts of Examples 32-42, i. e., where the metal acetate (or acetic acid) is replaced by other salts or anions, a modification of the procedure of Example 2 in view of the low water solubility of some of the reagent salts may be used. Ex-

ample 32 is illustrative of this modification and was as follows:

#### EXAMPLE 32 PROCEDURE

Four hundred grams of Sour Oil Treat 189 were charged into a 1-liter, four-necked, round-bottom flask

equipped with a mechanical stirrer, thermometer, air inlet tube, reflux condenser and dropping funnel. The sour oil was heated with stirring and with a moderate stream of air passing through it to approximately 75° C. A slurry of 24.7 grams (2.8 equivalents based on total acidity) of grease makers' lime in 75 ml. water was then added over a one-hour period in small increments through the dropping funnel. This was followed by the dropwise addition over a one-hour period of a solution containing 6.5 grams (0.6 equivalent) 98 per cent formic acid and 13.0 grams (0.6 equivalent) chloroacetic acid in 100 ml. water. The dehydration was effected by gradually heating the reaction mixture to 115° C. while removing the water with a Dean-Stark take-off. To insure the complete removal of the water, the temperature was maintained at 115° C. for one hour.

The filtration was carried out by stirring into the product 16 grams (4 per cent by weight of sour oil charged) of "Hyflo" filter aid and filtering this mixture through a heated Buchner funnel precoated with "Hyflo."

Analysis of product:

Per cent calcium=2.39 (150 per cent in excess of normal salt).  
Per cent sulfur=1.67  
Per cent chloride=1.05  
Kin. vis. @ 210° F.=48.0 cs.

The amount of complex salt product utilized in a lubricating oil will depend upon the particular oil and the application for which it is designed. Generally, amounts ranging from about 0.1 up to about 20 weight per cent may be used, the usual amount being from about 0.5 to about 10 weight per cent.

The complex salt products of this invention may be used in lubricating oil compositions containing other addition agents designed to improve the oil in different respects, e. g., antioxidants, extreme pressure agents, pour point depressants, viscosity index improvers, defoamants, etc.

Although the complex salts of this invention are intended primarily for use as lubricating oil additives, they are also adaptable for use in other applications, e. g., they find application in the manufacture of detergent soaps and are useful as dispersants and rust preventives. They may also be used as additives for cutting and textile oils.

Although the proportions and utility of certain specific representative complex salt products and oil compositions thereof have been described in detail herein, it is not intended that the invention be limited in any way thereby, but that it include such variations and procedures and such products and compositions as come within the spirit and scope of the accompanying claims.

We claim:

1. A complex metal salt of a hydrocarbon-soluble sulfonic acid produced by the method which comprises the steps of (1) forming a mixture of a hydrocarbon solution of the sulfonic acid with water and a reagent combination which will provide in said mixture at least about 1.6 equivalents of a metal hydroxide, at least about 0.6 equivalent of a metal formate and at least about 0.6 equivalent of an aliphatic metal carboxylate, other than a metal formate, having up to about 20 carbon atoms in the aliphatic portion thereof; the equivalents of said metal hydroxide, metal formate and metal carboxylate being based on the total equivalents of acid-hydrogen present in said hydrocarbon solution of the sulfonic acid and the metal constituent of said metal hydroxide, metal formate and metal carboxylate being a metal selected from groups I and II of the periodic table of the elements, (2) substantially completely dehydrating the reaction mixture formed in step 1 and (3) filtering off insoluble material.

2. A complex metal salt of a petroleum sulfonic acid produced by the method which comprises the steps of (1) intimately contacting an oil solution of the sulfonic

acid, in the presence of water, with at least about 1.6 equivalents of calcium hydroxide, at least about 0.6 equivalent of calcium formate and at least about 0.6 equivalent of calcium acetate, the equivalents of said calcium hydroxide, calcium formate and calcium acetate used being based on the total equivalents of acid-hydrogen present in said oil solution of the sulfonic acid, (2) substantially completely dehydrating the reaction mixture formed in step 1 and (3) filtering off insoluble material.

5 3. A complex metal salt of an oil-soluble synthetic wax-benzene sulfonic acid produced by the method which comprises the steps of (1) intimately contacting an oil solution of the wax-benzene sulfonic acid, in the presence of water, with at least about 1.6 equivalents of calcium hydroxide, at least about 0.6 equivalent of calcium formate and at least about 0.6 equivalent of calcium acetate, the equivalents of said calcium hydroxide, calcium formate and calcium acetate used being based on the total equivalents of acid-hydrogen present in said oil solution of the sulfonic acid, (2) substantially completely dehydrating the reaction mixture formed in step 1 and (3) filtering off insoluble material.

10 4. A complex metal salt of a petroleum sulfonic acid produced by the method which comprises the steps of (1)

25 intimately contacting an oil solution of the sulfonic acid, in the presence of water, with at least about 1.6 equivalents of calcium hydroxide, at least about 0.6 equivalent of calcium formate and at least about 0.6 equivalent of calcium propionate, the equivalents of said calcium hydroxide, calcium formate and calcium propionate used being based on the total equivalents of acid-hydrogen present in said oil solution of the sulfonic acid, (2) substantially completely dehydrating the reaction mixture formed in step 1 and (3) filtering off insoluble material.

30 5. A complex metal salt of a petroleum sulfonic acid produced by the method which comprises the steps of (1) intimately contacting an oil solution of the sulfonic acid, in the presence of water, with at least about 2.8 equivalents of magnesium hydroxide, at least about 0.6

35 equivalent of formic acid and at least about 0.6 equivalent of acetic acid, the equivalents of said magnesium hydroxide, formic acid and acetic acid used being based on the total equivalents of acid-hydrogen present in said oil solution of the sulfonic acid, (2) substantially completely dehydrating the reaction mixture formed in step 1 and (3) filtering off insoluble material.

40 6. A complex metal salt of a petroleum sulfonic acid produced by the method which comprises the steps of (1) intimately contacting an oil solution of the sulfonic acid, in the presence of water, with at least about 2.8 equivalents of barium hydroxide, at least about 0.6 equivalent of formic acid and at least about 0.6 equivalent of acetic acid, the equivalents of said barium hydroxide, formic acid and acetic acid used being based on the total equivalents of acid-hydrogen present in said oil solution of the sulfonic acid, (2) substantially completely dehydrating the reaction mixture formed in step 1 and (3) filtering off insoluble material.

45 7. A complex metal salt of a petroleum sulfonic acid produced by the method which comprises the steps of (1) intimately contacting an oil solution of the sulfonic acid, in the presence of water, with at least about 2.8 equivalents of barium hydroxide, at least about 0.6 equivalent of formic acid and at least about 0.6 equivalent of acetic acid, the equivalents of said barium hydroxide, formic acid and acetic acid used being based on the total equivalents of acid-hydrogen present in said oil solution of the sulfonic acid, (2) substantially completely dehydrating the reaction mixture formed in step 1 and (3) filtering off insoluble material.

50 8. A complex metal salt of a petroleum sulfonic acid produced by the method which comprises the steps of (1) intimately contacting an oil solution of the sulfonic acid with an aqueous reagent slurry containing at least about 1.6 equivalents of calcium hydroxide, at least about 0.6 equivalent of calcium formate and at least about 0.6 equivalent of calcium acetate, the equivalents of said calcium hydroxide, calcium formate and calcium acetate used being based on the total equivalents of acid-hydrogen present in said oil solution of the sulfonic acid, (2) substantially completely dehydrating the reaction mixture formed in step 1 and (3) filtering off insoluble material.

55 9. A complex metal salt of an oil-soluble synthetic wax-benzene sulfonic acid produced by the method which comprises the steps of (1) intimately contacting an oil solution of the wax-benzene sulfonic acid with an aqueous reagent slurry containing at least about 1.6 equivalents of

60 10 reagent slurry containing at least about 1.6 equivalents of

calcium hydroxide, at least about 0.6 equivalent of calcium formate and at least about 0.6 equivalent of calcium acetate, the equivalents of said calcium hydroxide, calcium formate and calcium acetate used being based on the total equivalents of acid-hydrogen present in said oil solution of the sulfonic acid, (2) substantially completely dehydrating the reaction mixture formed in step 1 and (3) filtering off insoluble material.

9. A complex metal salt of a petroleum sulfonic acid produced by the method which comprises the steps of (1) intimately contacting an oil solution of the sulfonic acid with an aqueous reagent slurry containing at least about 1.6 equivalents of calcium hydroxide, at least about 0.6 equivalent of calcium formate and at least about 0.6 equivalent of calcium propionate, the equivalents of said calcium hydroxide, calcium formate and calcium propionate used being based on the total equivalents of acid-hydrogen present in said oil solution of the sulfonic acid, (2) substantially completely dehydrating the reaction mixture formed in step 1 and (3) filtering off insoluble material.

10. A complex metal salt of a petroleum sulfonic acid produced by the method which comprises the step of (1) intimately contacting an oil solution of the sulfonic acid with an aqueous reagent slurry containing at least about 2.8 equivalents of magnesium hydroxide, at least about 0.6 equivalent of formic acid and at least about 0.6 equivalent of acetic acid, the equivalents of said magnesium hydroxide, formic acid and acetic acid used being based on the total equivalents of acid-hydrogen present in said oil solution of the sulfonic acid, (2) substantially completely dehydrating the reaction mixture formed in step 1 and (3) filtering off insoluble material.

11. A complex metal salt of a petroleum sulfonic acid produced by the method which comprises the steps of (1) intimately contacting an oil solution of the sulfonic acid with an aqueous reagent slurry containing at least about 2.8 equivalents of barium hydroxide, about 0.6 equivalent of formic acid and at least about 0.6 equivalent of acetic acid, the equivalents of said barium hydroxide, formic acid and acetic acid used being based on the total equivalents of acid-hydrogen present in said oil solution of the sulfonic acid, (2) substantially completely dehydrating the reaction mixture formed in step 1 and (3) filtering off insoluble material.

12. A mineral lubricating oil containing a minor proportion, sufficient to improve the detergent ability of said oil, of a complex metal salt of a hydrocarbon-soluble sulfonic acid produced by the method which comprises the steps of (1) forming a mixture of a hydrocarbon solution of the sulfonic acid with water and a reagent combination which will provide in said mixture at least about 1.6 equivalents of a metal hydroxide, at least about 0.6 equivalent of a metal formate and at least about 0.6 equivalent of an aliphatic metal carboxylate, other than a metal formate, having up to about 20 carbon atoms in the aliphatic portion thereof; the equivalents of said metal hydroxide, metal formate and metal carboxylate being based on the total equivalents of acid-hydrogen present in said hydrocarbon solution of the sulfonic acid and the metal constituent of said metal hydroxide, metal formate and metal carboxylate being a metal selected from groups I and II of the periodic table of the elements, (2) substantially completely dehydrating the reaction mixture formed in step 1 and (3) filtering off insoluble material.

13. A mineral lubricating oil containing a minor proportion, sufficient to improve the detergent ability of said oil, of a complex metal salt of a petroleum sulfonic acid produced by the method which comprises the steps of (1) intimately contacting an oil solution of the sulfonic acid, in the presence of water, with at least about 1.6 equivalents of calcium hydroxide, at least about 0.6 equivalent of calcium formate and at least about 0.6 equivalent of calcium acetate, the equivalents of said calcium hydroxide, calcium formate and calcium acetate used being

based on the total equivalents of acid-hydrogen present in said oil solution of the sulfonic acid, (2) substantially completely dehydrating the reaction mixture formed in step 1 and (3) filtering off insoluble material.

14. A mineral lubricating oil containing a minor proportion, sufficient to improve the detergent ability of said oil, of a complex metal salt of an oil-soluble synthetic wax-benzene sulfonic acid produced by the method which comprises the steps of (1) intimately contacting an oil solution of the wax-benzene sulfonic acid, in the presence of water, with at least about 1.6 equivalents of calcium hydroxide, at least about 0.6 equivalent of calcium acetate, the equivalents of said calcium hydroxide, calcium formate and calcium acetate used being based on the total equivalents of acid-hydrogen present in said oil solution of the sulfonic acid, (2) substantially completely dehydrating the reaction mixture formed in step 1 and (3) filtering off insoluble material.

15. A mineral lubricating oil containing a minor proportion, sufficient to improve the detergent ability of said oil, of a complex metal salt of a petroleum sulfonic acid produced by the method which comprises the steps of (1) intimately contacting an oil solution of the sulfonic acid, in the presence of water, with at least about 1.6 equivalents of calcium hydroxide, at least about 0.6 equivalent of calcium formate and at least about 0.6 equivalent of calcium propionate, the equivalents of said calcium hydroxide, calcium formate and calcium propionate used being based on the total equivalents of acid-hydrogen present in said oil solution of the sulfonic acid, (2) substantially completely dehydrating the reaction mixture formed in step 1 and (3) filtering off insoluble material.

16. A mineral lubricating oil containing a minor proportion, sufficient to improve the detergent ability of said oil, of a complex metal salt of a petroleum sulfonic acid produced by the method which comprises the steps of (1) intimately contacting an oil solution of the sulfonic acid, in the presence of water, with at least about 2.8 equivalents of magnesium hydroxide, at least about 0.6 equivalent of formic acid and at least about 0.6 equivalent of acetic acid, the equivalents of said magnesium hydroxide, formic acid and acetic acid used being based on the total equivalents of acid-hydrogen present in said oil solution of the sulfonic acid, (2) substantially completely dehydrating the reaction mixture formed in step 1 and (3) filtering off insoluble material.

17. A mineral lubricating oil containing a minor proportion, sufficient to improve the detergent ability of said oil, of a complex metal salt of a petroleum sulfonic acid produced by the method which comprises the steps of (1) intimately contacting an oil solution of the sulfonic acid, in the presence of water, with at least about 2.8 equivalents of barium hydroxide, at least about 0.6 equivalent of formic acid and at least about 0.6 equivalent of acetic acid, the equivalents of said barium hydroxide, formic acid and acetic acid used being based on the total equivalents of acid-hydrogen present in said oil solution of the sulfonic acid, (2) substantially completely dehydrating the reaction mixture formed in step 1 and (3) filtering off insoluble material.

18. A mineral lubricating oil containing a minor proportion, sufficient to improve the detergent ability of said oil, of a complex metal salt of a petroleum sulfonic acid produced by the method which comprises the steps of (1) intimately contacting an oil solution of the sulfonic acid with an aqueous reagent slurry containing at least about 1.6 equivalents of calcium hydroxide, at least about 0.6 equivalent of calcium formate and at least about 0.6 equivalent of calcium acetate, the equivalents of said calcium hydroxide, calcium formate and calcium acetate used being based on the total equivalents of acid-hydrogen present in said oil solution of the sulfonic acid, (2) substantially completely dehydrating the reaction mixture formed in step 1 and (3) filtering off insoluble material.

19. A mineral lubricating oil containing a minor proportion, sufficient to improve the detergent ability of said oil, of a complex metal salt of an oil-soluble synthetic wax-benzene sulfonic acid produced by the method which comprises the steps of (1) intimately contacting an oil solution of the wax-benzene sulfonic acid with an aqueous reagent slurry containing at least about 1.6 equivalents of calcium hydroxide, at least about 0.6 equivalent of calcium formate and at least about 0.6 equivalent of calcium acetate, the equivalents of said calcium hydroxide, calcium formate and calcium acetate used being based on the total equivalents of acid-hydrogen present in said oil solution of the sulfonic acid, (2) substantially completely dehydrating the reaction mixture formed in step 1 and (3) filtering off insoluble material.

20. A mineral lubricating oil containing a minor proportion, sufficient to improve the detergent ability of said oil, of a complex metal salt of a petroleum sulfonic acid produced by the method which comprises the steps of (1) intimately contacting an oil solution of the sulfonic acid with an aqueous reagent slurry containing at least about 1.6 equivalents of calcium hydroxide, at least about 0.6 equivalent of calcium formate and at least about 0.6 equivalent of calcium propionate, the equivalents of said calcium hydroxide, calcium formate and calcium propionate used being based on the total equivalents of acid-hydrogen present in said oil solution of the sulfonic acid, (2) substantially completely dehydrating the reaction mixture formed in step 1 and (3) filtering off insoluble material.

21. A mineral lubricating oil containing a minor proportion, sufficient to improve the detergent ability of said oil, of a complex metal salt of a petroleum sulfonic acid

produced by the method which comprises the steps of (1) intimately contacting an oil solution of the sulfonic acid with an aqueous reagent slurry containing at least about 2.8 equivalents of magnesium hydroxide, at least about 0.6 equivalent of formic acid and at least about 0.6 equivalent of acetic acid, the equivalents of said magnesium hydroxide, formic acid and acetic acid used being based on the total equivalents of acid-hydrogen present in said oil solution of the sulfonic acid, (2) substantially completely dehydrating the reaction mixture formed in step 1 and (3) filtering off insoluble material.

22. A mineral lubricating oil containing a minor proportion, sufficient to improve the detergent ability of said oil, of a complex metal salt of a petroleum sulfonic acid produced by the method which comprises the steps of (1) intimately contacting an oil solution of the sulfonic acid with an aqueous reagent slurry containing at least about 2.8 equivalents of barium hydroxide, at least about 0.6 equivalent of formic acid and at least about 0.6 equivalent of acetic acid, the equivalents of said barium hydroxide, formic acid and acetic acid used being based on the total equivalents of acid-hydrogen present in said oil solution of the sulfonic acid, (2) substantially completely dehydrating the reaction mixture formed in step 1 and (3) filtering off insoluble material.

## References Cited in the file of this patent

## UNITED STATES PATENTS

|    |            |            |       |               |
|----|------------|------------|-------|---------------|
| 30 | Re. 23,082 | Zimmer     | ----- | Jan. 25, 1949 |
|    | 2,467,176  | Zimmer     | ----- | Apr. 12, 1949 |
|    | 2,553,422  | O'Halloran | ----- | May 15, 1951  |
|    | 2,585,520  | Van Ess    | ----- | Feb. 12, 1952 |